# EUROPEAN PATENT SPECIFICATION

(11) **EP 1 270 438 B1**
(45) Date of publication and mention of the grant of the patent: **11.01.2012**
(21) Application number: 00981778.4
(22) Date of filing: 15.12.2000
(51) Int. Cl.: B65D 73/02, B65D 85/86

(54) **SHEET FOR EMBOSSED CARRIER TAPE**
FOLIE FÜR GEPRÄGTES TRÄGERBAND
FEUILLE DESTINE A UN RUBAN PORTEUR GAUFRE

(30) Priority: 15.12.1999 JP 35622899
(43) Date of publication of application: 02.01.2003
(73) Proprietor: DENKI KAGAKU KOGYO KABUSHIKI KAISHA, Chiyoda-ku, Tokyo 100-8455 (JP)
(72) Inventor: MIYAKAWA, Takeshi, Naganuma-cho, Isezaki-shi (JP); SHIMIZU, Mikio, Naganuma-cho, Isezaki-shi (JP)
(74) Representative: Hartz, Nikolai
(86) International application number: PCT/JP2000/008931
(87) International publication number: WO 2001/044070

(56) References cited:
- EP-A- 0 358 063
- JP-A- 7 076 390
- JP-A- 8 258 888
- US-A- 4 600 116
- US-A- 5 447 784
- US-A- 5 960 961

## Description

### TECHNICAL FIELD

The present invention relates to a sheet for an embossed carrier tape to be used as a material for an embossed carrier tape for packaging of e.g. chip components, IC or electronic components.

### BACKGROUND ART

Injection trays, vacuum-formed trays, magazines, embossed carrier tapes and the like are used for packaging of e.g. chip components, IC and electronic components, and particularly embossed carrier tapes are widely used with a purpose of conducting mounting efficiently. JP-A-P-7-76390 discloses an embossed carrier in accordance with the preamble of claim 1 of the present invention. Electronic components have become complicated, precise and downsized in recent years, and the speed of packaging and mounting of electronic components has also become high, and accordingly there is the problem that embossed carrier tapes are likely to break at the time of high speed mounting.

The present invention has been made to overcome the above problem. The present inventors have analyzed the mechanism of the breakage of embossed carrier tapes and as a result, have found that the breakage is caused by tearing from a flange corner portion or a sprocket hole portion of an embossed pocket. The present invention has been accomplished on the basis of this analysis.

### DISCLOSURE OF THE INVENTION

The present invention resides in a sheet for an embossed carrier tape according to claim 1 having a tear strength of at least 105 N/mm as defined in JIS (Japanese Industrial Standard)-K-7128-3.

### BEST MODE FOR CARRYING OUT THE INVENTION

Now, the present invention will be explained in detail below.

The sheet of the present invention has to have a tear strength of at least 105 N/mm as defined in JIS-K-7128-3, and it preferably has a tear strength of at least 115 N/mm. If the tear strength is less than 105 N/mm, when the sheet is used as an embossed carrier tape, the sheet is likely to break tear-wise from a sprocket hole portion or from a flange corner at the upper portion of the pocket.

The thickness of the sheet is not particularly limited so long as the tear strength is at least 105 N/mm as defined in JIS-K-7128-3, but is preferably within a range of from 0.1 to 3.0 mm. If the total thickness is less than 0.1 mm, the strength as a packaging container of the pocket portion to be obtained by forming the sheet tends to be inadequate, and if it exceeds 3.0 mm, forming such as air-pressure forming, vacuum forming or hot plate forming tends to be difficult.

The structure is not particularly limited and it may be a single-layer or a multi-layer consisting of at least two layers. A preferred structure is a single-layer one entirely having electrical conductivity. A structure having a base layer and an electrically conductive layer formed on at least one surface is also a preferred structure. Most preferred is a three-layer structure having an electrically conductive layer formed on both sides of the base layer.

The sheet of the present invention preferably has electrical conductivity on at least one side to be in contact with an electronic component. The sheet of the present invention is not necessarily electrically conductive depending upon the type of the electronic component to be stored, but the sheet is preferably electrically conductive so as to prevent breakdown of electronic components due to static electricity in many cases. The electrical conductivity of the surface is at most 10¹² Ω/□, preferably within a range of from 10¹² to 10⁴ Ω/□.

In order to impart electrical conductivity, a resin having electrical conductivity may be used for the electrically conductive layer, such as an electrically conductive resin comprising a thermoplastic resin and carbon black, an electrically conductive inorganic bulking agent, electrically conductive fibers and the like. Otherwise, an antistatic agent may be used for the surface or used together with the electrically conductive resin.

A thermoplastic resin may be used for the sheet of the present invention. The thermoplastic resin may, for example, be a polyvinyl chloride resin, a polyester resin, a polystyrene resin, an ABS resin, a polypropylene resin, a polyethylene resin, a polyphenylene ether resin or a polycarbonate resin, or a copolymer made mainly of styrene, ethylene, propylene, vinyl chloride or the like, and they may be used alone or in combination. Further, in a case of a multi-layer constitution comprising a surface layer, a base layer and a surface layer for example, it is possible to laminate different resins. To such a resin, in order to obtain electrical conductivity, an electrically conductive filler such as carbon black, an antistatic agent, a processing aid such as a plasticizer, a reinforcing agent, or a flatting agent or an inorganic filler may be added as the case requires.

As a method of processing the above-described thermoplastic resin into a sheet, a known extrusion or calendering may, for example, be employed, and to form the sheet into multi-layer, various means may be employed such as a feed block method by means of plural extruders, a multi-manifold method and an extrusion laminating method, a dry laminating method and gravure coating.

The sheet may be formed to be embossed by means of a forming method such as air-pressure forming, vacuum forming or hot plate forming to obtain an embossed carrier tape.

Now, the present invention will be explained in further detail with reference to Examples.

### EXAMPLE 1

Panlite L-1225 (manufactured by Teijin Chemicals Ltd.) which is a polycarbonate resin (referred to simply as PC in Table 1) and 20 wt% of Denka Black granules (acetylene black manufactured by Denki Kagaku Kogyo K.K.) which is carbon black (referred to simply as CB in Table 1) were preliminarily kneaded and pelletized by means of a φ50 mm vent type biaxial extruder to obtain an electrically conductive resin compound. Using said electrically conductive resin compound, and using a φ65 mm extruder (L/D=28) and a T-die having a width of 500 mm, a sheet having a thickness of 300 µm was obtained. Further, said sheet was slit into a width of 24 mm to obtain an embossed carrier tape having a pocket size of 12 mm x 15 mm x 5.5 mm and having a width of 24 mm by means of a carrier tape forming machine manufactured by EDG.

### EXAMPLE 2

As a surface layer resin, Panlite L-1225 (manufactured by Teijin Chemicals Ltd.) which is a polycarbonate resin and 12 wt% of Ketjenblack EC (manufactured by LION AKZO CO., LTD.) which is a carbon black were preliminarily kneaded and pelletized by means of a φ50 mm vent type biaxial extruder to obtain an electrically conductive resin compound. Using said electrically conductive resin compound and an ABS resin Techno ABS YT-346 (manufactured by TECHNOPOLYMER) for a sheet base layer, by means of a feed block method using a φ65 mm extruder (L/D=28), a φ40 mm extruder (L/D=26) and a T-die having a width of 500 mm, a three-layer sheet having a total thickness of 200 µm and a thickness of each electrically conductive resin composition layer of 30 µm was obtained. Using said sheet, an embossed carrier tape was obtained in the same manner as in Example 1.

### EXAMPLE 3

A sheet and an embossed carrier tape were obtained in the same manner as in Example 1 except that a polyethylene terephthalate resin (referred to simply as PET in Table 1) was used.

### EXAMPLE 4

A three-layer sheet having a thickness of 400 µm and a thickness of each electrically conductive resin composition layer of 30 µm was obtained in the same manner as in Example 2 except that as a surface layer resin, an electrically conductive resin compound obtained by preliminarily kneading and pelletizing Toyo Styrol E640N (manufactured by TOYO STYRENE) which is a polystyrene resin (referred to simply as PS in Table 1) and 12 wt% of Ketjenblack EC (manufactured by LION AKZO CO., LTD.) by means of a φ50 mm vent type biaxial extruder was used. Using said sheet, an embossed carrier tape was obtained in the same manner as in Example 2.

### EXAMPLE 5

A sheet having a thickness of 500 µm and an embossed carrier tape were obtained in the same manner as in Example 1 except that TP-URX (manufactured by Denki Kagaku Kogyo K.K.) which is a styrene-methyl methacrylate copolymer resin (referred to simply as MS in Table 1) was used.

### COMPARATIVE EXAMPLE 1

Toyo Styrol E640N (manufactured by TOYO STYRENE) which is a polystyrene resin and 18 wt% of Ketjenblack EC (manufactured by LION AKZO CO., LTD.) were preliminarily kneaded and pelletized by means of a φ50 mm vent type biaxial extruder to obtain an electrically conductive resin compound. A sheet and an embossed carrier tape were obtained in the same manner as in Example 1 except that said compound was used.

### COMPARATIVE EXAMPLE 2

A sheet having a thickness of 500 µm and an embossed carrier tape were obtained in the same manner as in Example 5 except that a styrene-methyl methacrylate copolymer resin TP-SX (manufactured by Denki Kagaku Kogyo K.K.) was used.

### COMPARATIVE EXAMPLE 3

A sheet and an embossed carrier tape were obtained in the same manner as in Example 4 except that as a base layer resin, a polystyrene resin Toyo Styrol HRM 20 (manufactured by TOYO STYRENE) was used.

### COMPARATIVE EXAMPLE 4

A sheet and an embossed carrier tape were obtained in the same manner as in Example 2 except that as a base layer resin, a polystyrene resin Toyo Styrol HRM 20 (manufactured by TOYO STYRENE) was used.

The tear strength of the obtained sheet was measured in accordance with JIS-K-7128-3, and the embossed carrier tape was subjected to a tensile test by means of an autograph tensile test with a chuck space of 32 mm at a tensile rate of 10 cm/min, and the evaluation results are shown in Table 1.

In Examples, a strength of the carrier tape of at least 60 N was obtained, whereas in Comparative Examples, it was less than 50 N. Further, with respect to each of the embossed carrier tapes of Examples and Comparative Examples, mounting test for emboss 100 pockets was carried out by using a mounting machine with a component mounting tact of 0.1 sec/component. In Examples, no problem arose such that the embossed carrier tape broke, whereas in Comparative Examples, a problem arose such that the embossed carrier tape broke.

**Table 1**

| Item | | Base layer | Surface layer | Sheet thickness | Tear strength | Carrier tape strength |
|---|---|---|---|---|---|---|
| (unit) | | | | (µm) | (N/mm) | (N) |
| Examples | 1 | PC+CB | | 300 | 162 | 109 |
| | 2 | ABS | PC+CB | 200 | 143 | 82 |
| | 3 | PET+CB | | 300 | 137 | 129 |
| | 4 | ABS | PS(E640N )+CB | 400 | 126 | 100 |
| | 5 | MS(TP-URX)+CB | | 500 | 117 | 64 |
| Comparative Examples | 1 | PS+CB | | 300 | 78 | 42 |
| | 2 | MS(TP-SX)+CB | | 500 | 82 | 45 |
| | 3 | ABS | PS(HRM-20)+CB | 300 | 64 | 38 |
| | 4 | PS(HRM20) | PC+CB | 200 | 72 | 35 |

### INDUSTRIAL APPLICABILITY

A sheet for an embossed carrier tape having a tear strength of at least 105 N/mm as defined in JIS-K-7128-3 is useful for high-speed mounting.

## Claims

1. An embossed carrier tape **characterised in that** it comprises a sheet having a tear strength of at least 105 N/mm as defined in JIS-K-7128-3.

2. The embossed carrier tape according to claim 1, wherein the sheet has a tear strength of at least 115 N/mm as defined in JIS-K-7128-3

3. The embossed carrier tape according to claim 1, wherein said sheet has a surface resistance of at least one surface of at most 10¹² Ω/□.

4. The embossed carrier tape according to claim 3, wherein said sheet is a single-layer sheet.

5. The embossed carrier tape according to claim 3, wherein said sheet is a multi-layer sheet.

6. The embossed carrier tape according to claim 5, wherein said sheet has a base layer and an electrically conductive surface layer.

7. The embossed carrier tape according to any one of claims 1 to 6, wherein said sheet uses a thermoplastic resin.

8. The embossed carrier tape according to claim 1, wherein said sheet uses a thermoplastic resin and has a base layer and a surface layer having a surface resistance of at most 10¹² Ω/□ on both sides of the base layer

9. The embossed carrier tape according to claim 1, wherein the thickness of the sheet is from 200 to 500 µm.

10. The embossed carrier tape according to claim 1, wherein a thermoplastic resin selected from a polycarbonate resin, an ABS resin, a polyethylene terephthalate resin, a polystyrene resin and a styrene-methyl methacrylate copolymer resin is used for said sheet.

## Patentansprüche

1. Geprägtes Trägerband, **dadurch gekennzeichnet, dass** es eine Folie mit einer Reißfestigkeit von mindestens 105 N/mm wie in JIS-K-7128-3 definiert aufweist.

2. Das geprägte Trägerband gemäß Anspruch 1, worin die Folie eine Reißfestigkeit von mindestens 115 N/mm wie in JIS-K-7128-3 definiert aufweist.

3. Das geprägte Trägerband gemäß Anspruch 1, worin die Folie einen Oberflächenwiderstand auf mindestens einer Oberfläche von höchstens 10¹² Ω/□ aufweist.

4. Das geprägte Trägerband gemäß Anspruch 3, worin die Folie eine einschichtige Folie ist.

5. Das geprägte Trägerband gemäß Anspruch 3, worin die Folie eine mehrschichtige Folie ist.

6. Das geprägte Trägerband gemäß Anspruch 5, worin die Folie eine Basisschicht und eine elektrisch leitfähige Oberflächenschicht aufweist.

7. Das geprägte Trägerband gemäß einem der Ansprüche 1 bis 6, worin die Folie ein thermoplastisches Harz verwendet.

8. Das geprägte Trägerband gemäß Anspruch 1, worin die Folie ein thermoplastisches Harz verwendet und eine Basisschicht und eine Oberschicht aufweist, und einen Oberflächenwiderstand von höchstens 10¹² Ω/□ auf beiden Seiten der Basisschicht.

9. Das geprägte Trägerband gemäß Anspruch 1, worin die Dicke der Folie 200 bis 500 µm beträgt.

10. Das geprägte Trägerband gemäß Anspruch 1, worin ein thermoplastisches Harz ausgewählt aus einem Polycarbonatharz, einem ABS-Harz, einem PolyethylenTerephthalat-Harz, einem Polystyrolharz und einem Styrol-Methylmethacrylat-Copolymer für die Folie verwendet wird.

## Revendications

1. Ruban porteur gaufré **caractérisé en ce qu'**il comprend une feuille présentant une résistance à la déchirure d'au moins 105 N/mm telle que définie dans la norme JIS-K-7128-3.

2. Ruban porteur gaufré selon la revendication 1, dans lequel la feuille présente une résistance à la déchirure d'au moins 115 N/mm telle que définie dans la norme JIS-K-7128-3.

3. Ruban porteur gaufré selon la revendication 1, dans lequel ladite feuille présente une résistance de surface d'au moins une surface d'au plus 10¹² Ω/□.

4. Ruban porteur gaufré selon la revendication 3, dans lequel ladite feuille est une feuille à une seule couche.

5. Ruban porteur gaufré selon la revendication 3, dans lequel ladite feuille est une feuille multi-couches.

6. Ruban porteur gaufré selon la revendication 5, dans lequel ladite feuille présente une couche de base et une couche de surface électriquement conductrice.

7. Ruban porteur gaufré selon l'une quelconque des revendications 1 à 6, dans lequel ladite feuille utilise une résine thermoplastique.

8. Ruban porteur gaufré selon la revendication 1, dans lequel ladite feuille utilise une résine thermoplastique et présente une couche de base et une couche de surface présentant une résistance de surface d'au plus 10¹²Ω/□ des deux côtés de la couche de base.

9. Ruban porteur gaufré selon la revendication 1, dans lequel l'épaisseur de la feuille est de 200 à 500 µm.

10. Ruban porteur gaufré selon la revendication 1, dans lequel une résine thermoplastique choisie parmi une résine de polycarbonate, une résine ABS, une résine de polyéthylène térephtalate, une résine de polystyrène et une résine de copolymère de styrène-méthacrylate de méthyle, est utilisée pour ladite feuille.
